

# UNITED STATES PATENT OFFICE.

FIN SPARRE, OF WILMINGTON, DELAWARE, ASSIGNOR TO THE E. I. DU PONT DE NEMOURS POWDER COMPANY, OF WILMINGTON, DELAWARE, A CORPORATION OF NEW JERSEY.

## EXPLOSIVE.

No. 850,502.

Specification of Letters Patent.

Patented April 16, 1907.

Application filed February 8, 1906. Serial No. 300,091.

*To all whom it may concern:*

Be it known that I, FIN SPARRE, a subject of the King of Norway, residing at Wilmington, county of Newcastle, and State of Delaware, have invented a new and useful Improvement in Explosives, of which the following is a full, clear, and exact description.

The object of my invention is to produce an explosive suitable for blasting and capable of acting as an effective substitute for the lower grades of dynamite, but having the advantage over dynamite of being safer and non-freezing.

My explosive consists, preferably, of the following ingredients: nitrocellulose, ammonium nitrate, a metallic ingredient, such as ferrosilicon or iron pyrites, sodium or potassium nitrate, and sulfur and charcoal or kerosene. Both the sodium nitrate and the potassium nitrate may be employed, one being the equivalent of the other, in my composition.

The following composition illustrates my invention and the proportions of the several ingredients:

|                        |                                             |
|------------------------|---------------------------------------------|
| Nitrocellulose.....    | 5 to 20 per cent., preferably 10 per cent.  |
| Ferrosilicon.....      | 5 to 20 per cent., preferably 10 per cent.  |
| Ammonium nitrate.....  | 25 to 75 per cent., preferably 40 per cent. |
| Sodium nitrate.....    | 10 to 50 per cent., preferably 30 per cent. |
| Potassium nitrate..... | 10 to 50 per cent., preferably 30 per cent. |
| Sulfur.....            | 2 to 8 per cent., preferably 4 per cent.    |
| Charcoal.....          | 0 to 8 per cent., preferably 3 per cent.    |
| Kerosene.....          | 0 to 8 per cent., preferably 3 per cent.    |

The foregoing ingredients are preferably incorporated in the ordinary way of making safety-powders. The simplest way of incorporating the ingredients is to place the ingredients in the described proportions while in a dry state in a rolling-mill or pulverizing-barrel such as is commonly employed in the manufacture of both black powder and safety-powders, the materials being pulverized and mixed by the action of the machine for approximately three hours.

The proportion of ammonium nitrate may be substantially decreased, and, indeed, it may be omitted altogether. If ammonium nitrate be omitted or its proportion substantially decreased, the proportion of nitrocellulose and also the proportion of sodium nitrate or potassium nitrate should be substantially increased.

The following is an example of a composition with ammonium nitrate omitted.

|                        |                                             |
|------------------------|---------------------------------------------|
| Nitrocellulose.....    | 15 to 60 per cent., preferably 30 per cent. |
| Ferrosilicon.....      | 5 to 25 per cent., preferably 11 per cent.  |
| Sodium nitrate.....    | 30 to 70 per cent., preferably 52 per cent. |
| Potassium nitrate..... | 30 to 70 per cent., preferably 52 per cent. |
| Sulfur.....            | 2 to 10 per cent., preferably 3 per cent.   |
| Charcoal.....          | 0 to 10 per cent., preferably 4 per cent.   |

Having now fully described my invention, what I claim, and desire to protect by Letters Patent, is—

1. An explosive composition containing nitrocellulose, ferrosilicon, sodium nitrate and sulfur in substantially the described proportions.
2. An explosive composition containing nitrocellulose, ferrosilicon and sodium nitrate in substantially the described proportions.
3. An explosive composition containing nitrocellulose, ferrosilicon, sodium nitrate, sulfur and charcoal in substantially the described proportions.
4. An explosive composition containing nitrocellulose, ferrosilicon, sodium nitrate, ammonium nitrate, sulfur and charcoal in substantially the described proportions.

In testimony of which invention I have hereunto set my hand, at Wilmington, on this 1st day of February, 1906.

FIN SPARRE.

Witnesses:

CHARLES G. GUYER,  
ALVIN B. ROBERSON.